

May 26, 1953

A. R. SLOMAN

2,639,987

TWO-STAGE PULPING PROCESS

Filed June 15, 1948

2 Sheets-Sheet 1



Fig. 1.



Fig. 2.

Inventor:  
Arthur Raymond Slobom

By Prince Scheffler & Parker,  
his Attorneys.

May 26, 1953

A. R. SLOMAN

2,639,987

TWO-STAGE PULPING PROCESS

Filed June 15, 1948

2 Sheets-Sheet 2



Fig. 3.

Inventor:  
Arthur Raymond Slobom

By Pierce, Schoffler & Parker.  
his Attorneys.

## UNITED STATES PATENT OFFICE

2,639,987

## TWO-STAGE PULPING PROCESS

Arthur Raymond Sloman, Burnie, Tasmania,  
Australia, assignor to Associated Pulp and  
Paper Mills Limited, Melbourne, Victoria, Aus-  
tralia, a corporation of Victoria

Application June 15, 1948, Serial No. 33,035  
In Australia July 9, 1947

1 Claim. (Cl. 92—13)

1

This invention relates to improvements in the production of paper pulp and refers especially to improvements in the cooking of wood by the alkaline processes for the production of paper pulp. The invention is applicable to the soda process or sulphate (kraft) process but is particularly applicable to the former.

The general practice in alkaline digesting processes for isolating cellulose pulps from wood or other cellulose-bearing raw materials has been to cook these materials in a single-stage cook, the active chemical being added either at the commencement of the cook or by injection under pressure during the course of the cook. There have been developments towards multi-stage alkaline cooking of cellulosic materials for the production of pulps, but these processes have not been entirely satisfactory, they have not effected the desired economies in operation, in some instances they require cumbersome operating procedures, and in most cases they have required the addition of some new caustic soda in each stage of the process.

I have discovered that it is possible to produce easy-bleaching pulps from wood by the use of a two-stage process in which the effluent liquor from the second stages is used in the first stages of subsequent cooks, without the addition of any substantial quantity of new active chemical (e. g. caustic soda as "white liquor") in the first stage treatments. By this means considerable savings can be effected in the amount of active chemical required to produce pulps with the same characteristics.

In this specification the term "white liquor" is used to refer to a solution containing recovered alkali and/or fresh alkali in such concentration as to render the solution suitable for the alkaline pulping of wood, and the term "black liquor" is used to refer to the liquor discharged from the digester after the alkaline cooking and delignification of wood and which contains both free alkali and alkali combined with organic materials dissolved from the wood.

In this specification the "Permanganate number" of a pulp is defined as the number of millilitres of decinormal potassium permanganate reduced by 1.000 gms. oven-dry pulp in five minutes when the pulp is treated with the permanganate according to the test conditions specified below:

The equivalent of 1.000 gms. O. D. pulp is dispersed in 180 mls. of distilled water at 20° C. 20 mls. 10% sulphuric acid is added followed by 50 mls. of tenth normal potassium permanganate solution. The reaction is held at 20° C. and carried out with constant stirring for exactly five minutes after the addition of the permanganate. At the end of the reaction period 50 mls. of tenth normal ferrous ammonium sul-

phate (acidified with 100 mls. concentrated sulphuric acid per litre of solution) is added to stop the reaction. The excess of ferrous ammonium sulphate is then back-titrated with tenth normal potassium permanganate. The number of millilitres of potassium permanganate solution required for the back-titration is the permanganate number of the pulp.

Where the permanganate number of the pulp exceeds 20 when carried out according to the above method the volume of potassium permanganate solution, sulphuric acid, water and ferrous ammonium sulphate are increased until the ratio of volume of permanganate added to volume of permanganate reduced is not less than 2.5. The ratio of volume of permanganate added, to volume of 10% sulphuric acid, to volume of water is held constant at 5:2:18 when such changes in the method are necessary."

I have found experimentally that the black liquor obtained from normal single stage alkaline cooks (in which caustic soda, either alone or in conjunction with sodium carbonate or sodium sulphide, is the active chemical) contains substantial quantities of unneutralized caustic soda and other caustic alkalinity. In fact, it has been ascertained that in cooking *Eucalyptus gigantea* by the soda process in a normal single stage cook with a soda charge of, for example, 24% NaOH on the O. D. wood (oven-dry wood), only about 14% NaOH on the O. D. wood is neutralized by the wood. With *Pinus radiata* a conifer commonly known as "Monterey pine" about 17% NaOH is neutralized with a soda charge of 34% NaOH/O. D. wood. Similar results with other woods are listed below:

TABLE 1

| Wood Species                              | Soda Charge, Percent NaOH/O. D. Wood | Soda Neutralized, Percent NaOH/O. D. Wood |
|-------------------------------------------|--------------------------------------|-------------------------------------------|
| <i>Nothofagus cunninghamii</i> (white)    | 18-22                                | 13.5                                      |
| <i>Nothofagus cunninghamii</i> (red)      | 20-24                                | 13.6                                      |
| <i>Pomaderris smithii</i>                 | 20-26                                | 14.9                                      |
| <i>Eucalyptus obliqua</i> (age 100 years) | 24-28                                | 16.0                                      |

The common name of *Nothofagus cunninghamii* is "myrtle" and *Pomaderris smithii* is known commonly as "dogwood"; both are deciduous trees.

In these experiments the NaOH remaining in the black liquor was determined potentiometrically.

The use of different soda charges with the one wood, providing the soda charge is in excess of that equivalent to the amount shown to be neutralized in the cook, does not materially affect the amount of caustic soda neutralized in the cook when pulps of the same bleach requirement

(indicated by the permanganate number) are produced from the one wood. Over the ranges of soda charge shown in Table 1 for each wood, the amount of soda neutralized was constant at the amount shown in the table for that wood. In all cases the pulps produced had permanganate numbers close to 15.

It appears possible that the main function of the additional caustic soda used over the amount neutralized is to provide a greater mass of caustic soda in order to increase the speed of the delignification process, or alternatively that the physico-chemical condition of the wood is affected in a way which improves the rate of diffusion of the sodium lignin complex from the fibers and intercellular zones. Thus in pulp mills where single stage alkaline cooking is practised, substantial quantities of unneutralized alkali are returned to the alkali recovery system. In this system the caustic soda is converted to sodium carbonate and then requires to be recausticised.

depress the rate of lignin removal, or, in the case of cooks conducted for a given time, to result in the production of pulps having higher permanganate numbers.

A series of experiments was carried out by cooking a sample of *Eucalyptus gigantea* with increasing amounts of black liquor, and maintaining constant the charge of caustic soda added by way of white liquor. All the cooks were charged with 20% NaOH/O. D. wood added as white liquor, and the liquor ratio (i. e. mls. liquor/gms. O. D. wood) was made up to 5:1 by the addition of either black liquor or water or both, and in one case by the addition of more highly concentrated black liquor. The cooks were heated to 170° C. over a period of two hours and held at this temperature for a period of two hours. The cooks were then shock-cooled by being placed in cold water. The conditions used and the results obtained are shown in the table below:

TABLE 2

| Cook No. | Liquor                                                                                                                                                                               | Black Liquor solids added in liquor, gms./100 gms. O. D. wood | Permanganate No. of pulp | Pulp yield (unbleached), percent on O. D. wood | Total free soda added, gms. NaOH | Soda neutralized during cook, percent NaOH/O. D. wood |
|----------|--------------------------------------------------------------------------------------------------------------------------------------------------------------------------------------|---------------------------------------------------------------|--------------------------|------------------------------------------------|----------------------------------|-------------------------------------------------------|
| 1.....   | 121 mls. white liquor containing 20.0 gms. NaOH and 360 mls. distilled water.                                                                                                        | Nil.....                                                      | 14.5.....                | 52.5.....                                      | 20.0                             | 13.0                                                  |
| 2.....   | 121 mls. white liquor (as above), 250 mls. black liquor, 110 mls. distilled water.                                                                                                   | 103.5.....                                                    | 16.3.....                | 53.1.....                                      | 25.6                             | 13.0                                                  |
| 3.....   | 121 mls. white liquor (as above), 350 mls. concentrated black liquor containing 160 gms. black liquor solids obtained by evaporating 770 mls. of black liquor (as above) to 350 mls. | 320.....                                                      | approx. 51.              | approx. 60.                                    | 37.2                             | 13.2                                                  |

thereby greatly increasing cost without doing more useful work than increasing reaction rate.

Now, the black liquor thus normally returned to the recovery system is not useful alone for further single stage cooking owing, firstly, to the relatively low concentration of free alkali, and secondly, to the presence of high concentrations of wood solids (e. g. lignin, hemi-celluloses and other organic materials).

I have found, however, that the black liquor can be used as a source of soda for neutralizing much of the natural acidity in wood and thereby reducing the quantity of new caustic soda required in the pulping process.

From my experiments, it appears that black liquor can only be used effectively for this purpose if the cook is carried out in two stages with the addition of black liquor alone or together with relatively small amounts of other alkali in the first stage.

In normal single-stage cooking, it is known to employ black liquor from previous cooks as liquor make-up to cover the charge of wood. It is recognised that the free or loosely combined caustic soda in this liquor when used according to normal practice cannot be regarded as behaving as part of the active chemical charged to the cook, either for the purpose of neutralising wood acids or for effecting delignification, in that the cooking time required to produce a pulp of given permanganate number is not reduced by increasing the proportion of black liquor used, while still maintaining a constant charge of active NaOH added as white liquor. In fact, the presence of wood solids in the black liquor tends to

The black liquor used in the above experiments contained 207.5 g. p. l. of total solids and 22.4 g. p. l. caustic alkalinity expressed as NaOH.

It can be seen from Table 2 that the addition of black liquor tended to result in the production of pulps with higher permanganate numbers, although the amount of soda neutralized was substantially constant. This is probably due to the presence of substantial amounts of wood solids (lignin hemicelluloses and the like) in solution in the black liquor, the effect of which is to more than counteract the increase in rate of delignification which would be expected to follow from the increase in active alkali concentration obtained by the addition of black liquor.

The presence of wood solids in solution appears to have the effect of preventing diffusion and/or dissolution of the material of the wood, even though this material has reacted chemically with the normal amount of caustic soda.

I have also discovered that the neutralization of natural acidity in wood can be carried out with solutions of relatively low alkali concentration, and that this process does not appear to be adversely affected by the presence of wood solids in the liquor. It is possible to neutralize up to about 10% NaOH on O. D. wood (*Eucalyptus gigantea*) and probably higher amounts in the case of woods having a higher content of acidic materials, using liquors weak in alkali (i. e. in concentrations less than, say, 40 gms. per litre with a liquor ratio of, say, 3.5 to 1) and carrying substantial quantities of wood solids.

It has also been found that if the cooking or digesting treatment of wood is conducted in two

stages, the first essentially a process for neutralizing natural acidity, and the second essentially a delignifying process, the total alkali neutralized over both stages is substantially the same as would be neutralized in a single stage cook conducted to give pulp with the same bleachability (i. e. permanganate number). That is, if in a single stage soda cook on *Eucalyptus gigantea* conducted at say 170° C. using 24% NaOH on O. D. wood to give pulp with permanganate number 15, 14% NaOH on the O. D. wood were neutralized, then in a two-stage cook on the same wood where in the first stage 10% NaOH on O. D. wood is neutralized approximately 4% would be neutralized in the second stage if pulp having the same permanganate number is produced. The black liquor from this second stage cook then contains substantially the same concentration of unneutralized caustic alkalinity as that from the single stage cook employing 24% NaOH on O. D. wood.

This invention, then, is based on these findings and provides a means whereby appreciable savings in the amounts of fresh alkali required for cooking wood and like materials can be effected.

An important feature of the invention resides in using the liquor from the second stage of a two-stage cooking treatment to provide the alkali necessary for neutralizing the natural acidity of wood in a subsequent first stage treatment.

The invention broadly includes a two-stage alkaline process for the production of paper pulp from wood which comprises subjecting a wood charge to a first-stage digestion treatment to substantially neutralize its natural acidity, by cooking the wood in a closed vessel in black liquor at a temperature between 150° C. and 180° C., the caustic alkalinity of the black liquor used in said first-stage treatment being between 5% and 16% (expressed as NaOH on oven-dry wood) and from 80% to about 100% of said alkalinity being neutralized in said treatment, separating the resulting substantially exhausted liquor from the wood charge, and then subjecting the wood charge to a second-stage delignification treatment by cooking the wood charge in a closed vessel in a digestion liquor comprising white liquor at a temperature between 150° C. and 180° C. to produce a pulp, the caustic alkalinity of the digestion liquor used in the second-stage treatment being such that the caustic alkalinity of the black liquor separated from the wood charge after the said second-stage treatment is less than RP/Q lbs. NaOH per gallon where

R=alkali charge (as per cent NaOH on oven-dry wood) at which 80% of the alkali is neutralized by wood in a first-stage treatment,

P=concentration of caustic alkalinity in the black liquor leaving the second stage divided by the concentration of caustic alkalinity in the liquor after dilution,

Q=volume of black liquor charged to first-stage treatment (in gallons per 100 lbs. oven-dry wood).

The method of calculating, by means of the above mentioned formula, the maximum quantity of caustic alkalinity to be used in the second-stage treatment, will be more fully explained later in this specification.

Black liquor may also be added as "make-up" liquor in the second-stage treatment to make up the required volume, as in normal single stage cooking.

The process is carried out in a closed vessel,

such as a digester of the type normally used in the alkaline pulping of wood, and the temperature of the charge is preferably raised during the cooking treatments to a value between 150° C. and 180° C. Excellent results have been obtained using a maximum cooking temperature of 170° C. An elevated maximum temperature is particularly necessary in the first-stage treatment in order to secure full or substantial neutralization of the residual caustic alkalinity of the black liquor used in such treatment.

In the above temperature range, the time of the first-stage cooking is between 0.1 and 1.5 hours at maximum temperature. Treatment for about 0.25 hour at maximum temperature of 170° C. will normally be found sufficient in the first stage and if a lower maximum temperature is used a longer period of treatment will be necessary.

The cooking time in the second stage at a maximum temperature of 170° C. is normally between 1.0 and 3.0 hours, and is preferably about 2.0 hours.

The process is controlled in such a way that the free caustic alkalinity added to the first stage by way of the black liquor is between 5% and 16% expressed as NaOH on O. D. wood, and is preferably between 8% and 13%.

The amount of alkali added in first stage treatments by way of the black liquor will vary with the woods in use, and in most cases, it is desirable that the amount of caustic alkalinity should be between 60% and 75% of the alkali required to neutralize the natural acidity in the wood when the latter is cooked in a single stage cook to give pulp of the bleachability required. Thus with *Pinus radiata*, a wood requiring a relatively high alkali charge under normal operating conditions, the amount of caustic alkalinity introduced by way of black liquor should preferably be between 10% and 13%, expressed as NaOH on O. D. wood. With *Eucalyptus gigantea* the relative figures would be 8 to 10%.

The alkali addition in the first and second stage treatments is also controlled so that at least 80% of the caustic alkalinity of the black liquor used is neutralized in the first stage treatment. The method of control necessary to ensure this is described more fully later in this specification.

I have discovered that the liquor discharged from the first stage treatment is particularly suitable for the recovery of the lignin and other organic materials therefrom.

A further feature of the invention resides in the fact that, by means of this process the output of pulp may be increased for a given alkali consumption. In other words, in a mill having a certain soda recovery and causticisation capacity, and if, adequate digestion capacity is available, it is possible to substantially increase the output of pulp from the mill. This application of the process involves an increase in the ratio of wood solids to inorganic materials in the black liquor passed to the recovery system, and consequently an increase in evaporating and roasting capacity may be necessary if the pulp output is increased.

However, this is usually preferable to increasing the causticising and soda recovery plant since the operating costs of the latter are high and labour difficulties associated with its operation are considerable. Moreover, an increase in the wood solids content of the black liquor is advantageous in that it improves the burning qualities of the evaporated liquor.

According to a still further feature of the in-

vention, pulp produced by the two-stage process of this invention operating on a given time cycle possesses certain improved physical characteristics compared with pulp produced by the normal single stage process operating on the same time cycle.

A still further feature resides in the fact that in the process of this invention variations in cooking time required to give pulp of constant permanganate number (i. e. bleachability) consequent upon uncontrollable changes in alkali charge (per cent alkali on O. D. wood) are much less and affect the cooking cycle by a smaller time than is the case with normal single stage cooking.

I have ascertained by experiment that in soda pulping the graph of soda charge (per cent NaOH on O. D. wood) against the reciprocal of the time of cooking to produce at any one maximum temperature pulps of given permanganate number is substantially a straight line with positive slope in relation to the X-axis (soda charge). Hence, where the cooking time is relatively short, as in the second stage of the process of the present invention, a given variation in soda charge due to uncontrollable factors (e. g. variations in moisture content of wood charged) will necessitate substantially less change in cooking time, to produce pulp of required permanganate number, than where the cooking time is relatively longer, as in the normal single stage process, operating on the same time cycle.

In Figure 1 of the accompanying drawings is shown a flow sheet illustrating the normal single-stage cooking treatment for the production of pulp by the soda process, and in Figure 2 of the drawings is shown a flow sheet illustrating the two-stage process of this invention.

In Figure 2 the full lines indicate the first stage treatment and the dotted lines indicate the second-stage treatment.

Figure 3 is a graph showing quantity of caustic soda used in the treatment of wood against quantity neutralized and is referred to more fully later in this specification.

#### Example 1

The following is an example, for comparison purposes, of a normal single stage alkaline cooking treatment on *Eucalyptus gigantea* wood to produce a pulp having a permanganate number of about 15:

113 gms. of air dried wood (*Eucalyptus gigantea*) containing 100 gms. oven-dry wood was cooked with sufficient white liquor to give a soda charge of 24% NaOH on O. D. wood at a liquor ratio (i. e. mls. liquor/gms. O. D. wood) of 5.0 to 1. The temperature was raised to 170° C. over a period of 1.9 hours and the cook held at 170° C. for 1.28 hours. The permanganate number of the pulp was 14.9 and the concentration of caustic alkalinity in the black liquor was 20.6 gms. per litre (expressed as NaOH).

#### Example 2

The following is an example of a two-stage cooking treatment according to this invention on the same type of wood to produce a pulp having approximately the same permanganate number (i. e. 15):

113 gms. of air-dry wood (*Eucalyptus gigantea*) containing 100.0 gms. oven-dry wood were charged to a digester with 500 mls. of black liquor obtained from a previous soda cook and containing 23.4 g. p. l. of caustic alkalinity expressed as

grams NaOH per litre. The cook was heated to 170° C. over a period of 1.9 hours and the digester held at this temperature for 0.25 hour. The digester was then shock-cooled by cold water and the liquor effluent from this impregnation treatment titrated potentiometrically to determine the amount of caustic alkalinity which had been neutralized. This liquor contained 7.6 g. p. l. caustic alkalinity. Thus the wood had neutralized 7.9 gms. caustic alkalinity expressed as equivalent NaOH.

The liquor was drained from the wood and white liquor added to the digester in sufficient quantity to provide 16.1% NaOH (i. e. 24.0 minus 7.9) on the wood. This second stage was carried out by heating to 170° C. over a period of 1.9 hours and this temperature was held for 1.28 hours. The cook was shock-cooled in water and the pulp obtained had a permanganate number of 15.4. The black liquor from this stage contained 22.5 g. p. l. of caustic alkalinity expressed as NaOH, and 310 mls. of black liquor were recovered. Two cooks were conducted under these conditions to provide sufficient black liquor for the treatment described in Example 3.

#### Example 3

The black liquor from the second stage treatment of Example 2 was used to treat new wood in the following manner:

113 gms. of air-dry wood (*Eucalyptus gigantea*) containing 100 gms. of O. D. wood were treated with 500 mls. of black liquor from the second stage of the treatments described in Example 2 above. The liquor ratio was thus 5.1 to 1. After treatment at 170° C. for 0.25 hour and shock-cooling, the concentration of caustic alkalinity in the liquor was 7.6 g. p. l. (expressed as NaOH). Thus acidity in the wood equivalent to 7.4% NaOH on O. D. wood had been neutralized.

A second-stage treatment was then carried out with the addition of white liquor to the charge to give 16.6% NaOH (24.0 minus 7.4) on the O. D. wood. It was cooked at 170° C. for 1.28 hours, and the permanganate number of the pulp obtained was 15.6. The concentration of caustic alkalinity in the black liquor from this second stage was 22.9 g. p. l. (as NaOH).

#### Example 4

113 gms. of air-dry wood (*Eucalyptus gigantea*) containing 100 gms. of O. D. wood were treated with 500 mls. of black liquor obtained from a previous soda cook and containing 20.3 g. p. l. of caustic alkalinity expressed as grams NaOH per litre. The cook was heated to 170° C. over a period of 1.9 hours and the digester held at this temperature for 0.25 hour. The digester was then shock-cooled in water and the liquor from this impregnation treatment titrated potentiometrically to determine the amount of caustic alkalinity which had been neutralized. This liquor contained 5.66 g. p. l. caustic alkalinity. Thus the wood had neutralized 7.3 gms. caustic alkalinity expressed as equivalent NaOH.

The free liquor was drained from the wood and 150 mls. of liquor remained entrained in the wood. The liquor charged to the second stage was made up as follows:

White liquor (111.4 g. p. l. NaOH) \_\_\_\_ mls. 150  
Black liquor 20.3 g. p. l. free NaOH) \_\_\_\_ mls. 200

Thus the liquor ratio was 5:1 and 16.7% NaOH (24.0 minus 7.3) on O. D. wood was added as white liquor.

This second stage treatment was carried out by heating to 170° C. over a period of 1.9 hours, and this temperature was held for 1.28 hours. The cook was shock-cooled in water, and the pulp obtained had a permanganate number of 14.6. The black liquor from this stage contained 27.9 g. p. l. of caustic alkalinity expressed as NaOH.

*Example 5*

The following is an example of the process of this invention as applied to the sulphate or kraft process.

Wood charged 100 gms. O. D. *Eucalyptus gigantea*.  
Liquor ratio 4.5:1.  
Total alkali charged expressed as NaOH/O. D. wood. 22% on O. D. wood.  
Sulphidity 25%.  
Time to heat to maximum temperature 1.9 hours.  
Time at maximum temp 1.25 hours.  
Maximum cooking temp 170° C.  
Permanganate number of unbleached pulp 14.9.  
Caustic alkalinity of black liquor as NaOH 16.1 g. p. l.

A sample containing 78.6 gms. O. D. wood (*Eucalyptus gigantea*) was treated with 275 mls. of black liquor from a previous single-stage cook conducted under the conditions shown above. The liquor charged contained 16.1 g. p. l. caustic alkalinity expressed as NaOH. The cook was heated to 170° C. over a period of 1.9 hours and held at this temperature for 0.50 hour. The digester was then shock-cooled in water and the liquor drained from the wood. The liquor was titrated potentiometrically and the amount of caustic alkalinity remaining in the liquor was nil. Thus the wood had neutralized 5.65% NaOH on the O. D. wood.

The second stage was charged with white liquor containing 16.35% total alkali (NaOH and Na<sub>2</sub>S) expressed as NaOH, and the sulphidity of this liquor was 25%. The liquor ratio was made up to 4.5:1 by the addition of water.

The digester was heated to 170° C. over a period of 1.9 hours and held at this temperature for 1.25 hours. The cook was shock-cooled in cold water and the pulp obtained had a permanganate number of 12.0. The black liquor effluent from this stage contained caustic alkalinity equivalent to 14.0 g. p. l. expressed as NaOH.

*Example 6*

The following is a plant scale example of the process, using soda cooking.

Sufficient wood (mixed species of *Eucalyptus*) was charged to fill a digester having a volumetric capacity of 2650 cubic feet. The amount of wood charged was equivalent to about 30,000 lbs. O. D. wood. 9,000 gallons of black liquor from previous soda cooks, and containing approximately 23.0 g. p. l. caustic alkalinity, expressed as NaOH, was added. The digester was heated to 170° C. over a period of 2.0 hours by means of an external steam heater through which liquor, withdrawn from the bottom of the digester, was passed and returned to the top of the digester. The mass was held at 170° C. for 0.25 hour and the free liquor was then released from the digester by way of a valve and pipeline, the entrance to which was situated beneath screen plates in the bottom of the digester. The liquor leaving the digester con-

tained 3.0 g. p. l. caustic alkalinity expressed as NaOH, and had a pH of 9.3. The amount of soda neutralized was of the order of 6.0% NaOH/O. D. wood. 87% of the caustic alkalinity of the black liquor was neutralized in the first stage treatment.

After the liquor had been released steam was allowed to escape in the normal manner of "gassing down," as practised in the industry, and when the pressure of the system was in equilibrium with the atmosphere (at about 100° C.) sufficient white liquor was added to supply 16% NaOH/O. D. wood. For this purpose 4,000 gallons were required, and the total volume of liquor added was made up to 7,000 gallons by the addition of black liquor. Heating was recommenced and the mass was raised to a temperature of 170° C. over a period of 1.5 hours, and was held at this temperature for 2.5 hours.

The cook was then "gassed down" by the release of steam from the top of the digester, and when a gauge pressure of 80 lbs./sq. inch was reached, the digester was blown. The permanganate number of the pulp produced was 14 and the black liquor discharged with the pulp contained 40 g. p. l. of NaOH. This liquor was diluted in the blow tank with black liquor from the pulp washers, as shown in Fig. 1, and the mixed black liquor was further diluted during washing operations. The liquor leaving the washing system contained about 23 g. p. l. caustic alkalinity expressed as NaOH.

In comparing the time-cycle of the process of this invention with that of the normal single-stage process it may be assumed that, in the commercial application of the process, the time to fill the digester is 1 hour, the time for draining the liquor from the digester after completion of the first stage treatment and recharging with liquor for the second stage treatment is 1.5 hours, and the time for blowing the digester at the end of the cook is 0.25 hour.

Under these conditions the comparative times of a normal single-stage cook and of the two-stage process of this invention may be illustrated by the following table:

TABLE 3

*Single-stage treatment*

|                                     | Hours       |
|-------------------------------------|-------------|
| Time to fill                        | 1.00        |
| Time to heat to maximum temperature | 1.90        |
| Time at maximum temperature         | 5.00        |
| Time to blow                        | 0.25        |
| <b>Total</b>                        | <b>8.15</b> |

*Two-stage treatment*

|                                     | Hours       |
|-------------------------------------|-------------|
| First stage:                        |             |
| Time to fill                        | 1.00        |
| Time to heat to maximum temperature | 1.90        |
| Time at maximum temperature         | 0.25        |
| Second stage:                       |             |
| Time to drain and recharge          | 1.50        |
| Time to heat to maximum temperature | 1.90        |
| Time at maximum temperature         | 1.28        |
| Time to blow                        | 0.25        |
| <b>Total</b>                        | <b>8.08</b> |

It will be seen, therefore, that the two-stage treatment of this invention may be carried out on the same time cycle as the normal single-stage process, and the same pulp output may

thus be obtained by the process of this invention with substantial reduction in alkali consumption.

Thus, in a single stage cook using *Eucalyptus gigantea*, on an 8-hour cycle, the maximum cooking temperature being 170° C. and the pulp produced having a permanganate number of 15, the new alkali required was 18.6% NaOH on O. D. wood, whereas in the two-stage process of this invention as carried out in Examples 2 and 3 above, the new alkali consumption was 16.6% and 16.1% (NaOH on O. D. wood), respectively.

I have ascertained that the time required in the second stage of a two-stage cooking treatment according to this invention is substantially the same as is required in a normal single stage cook in which the soda charge is the same as the total soda charged over both stages in the two-stage treatment. That is, if the time required at 170° C. to give pulp with permanganate number 15 using 24% NaOH on the O. D. wood in a normal single stage cook is 1.28 hours, then in a two-stage cooking treatment according to this invention where 8% NaOH on the O. D. wood is neutralized in the first stage, the second stage using a soda charge of 16% NaOH and producing at 170° C. a pulp of permanganate number 15 will require 1.28 hours.

It will be clear to those skilled in the art that if the soda charge in the second stage of the process is increased, thereby reducing the cooking time, the black liquors from these stages will contain greater concentrations of unneutralized alkali, and that a point will be reached where the amount of soda available from these liquors will exceed that which can be neutralized in first stage treatments. If the soda charge in the second stage is reduced the cooking time required in the second stage is increased and the concentration of caustic alkalinity in the black liquor from this stage is reduced. A point will be reached where all the free alkali can be neutralized very easily in the first stage treatments, but this is offset by the longer cooking time required in the second stage. I have found that it is desirable that the amount of soda charged to the second stage should be controlled so that the concentration of caustic alkalinity remaining in the black liquor from this stage is below a figure which will permit the neutralization of at least 80% of this alkali in subsequent first stage treatments.

If the wood will neutralize at a maximum the equivalent of, say,  $x\%$  NaOH on the wood from black liquor in a first stage treatment, the optimum conditions under which to operate the process are those giving black liquor from the second stage containing a concentration of caustic alkalinity such that in normal operation approximately  $x\%$  NaOH on the wood is charged to first stage treatments. This will then mean that the time of cooking in the second stage is at a minimum consistent with the neutralization of the maximum amount of caustic alkalinity in the first stage.

If the residual alkalinity in the black liquor from the second stage treatments is greater than  $x\%$  NaOH on the wood, the excess alkali unneutralized in the first stage will be carried through to the soda recovery system, thereby increasing recovery costs, while if the residual alkalinity is less than  $x\%$  the time of cooking in the second stages will be unnecessarily prolonged.

The control of the system to achieve this end may be carried out as follows.

The wood to be used is tested by treating samples containing known O. D. weights of wood with increasing amounts of caustic soda over the range of, say, 6% to 14% as NaOH/O. D. wood, and with a fixed liquor ratio. The laboratory experiments are carried out by heating the reaction mixture at the same rate and for the same time at maximum temperature as would be used in a normal first stage treatment under mill conditions. After shock cooling at the conclusion of the first stages the liquors from these experiments are analysed by potentiometric titration to determine the residual caustic alkalinity remaining in the liquor, and from these results the percentage of the soda which had not been neutralized is calculated. The curves obtained by plotting soda applied (X axis) against percentage of soda neutralized (Y axis) are of the form shown in Figure 3. From these curves it can be seen that, with increasing soda charge, the percentage of the charge neutralized decreases progressively. For the purposes of this work we regard a minimum of 80% neutralization as being desirable, and on this basis would regard the soda charge at which 80% of the soda is neutralized (i. e. "R" % NaOH on O. D. wood) as being the greatest amount that should be added in first stage treatments with the wood under consideration. Hence "R" equals alkali charge (as per cent NaOH on O. D. wood) at which 80% of the alkali is neutralized by the wood in a first stage treatment.

In the flowsheet shown in Figure 2, it can be seen that black liquor leaving the digester with the pulp after the second stage will suffer some dilution during pulp washing operations. The amount of dilution occurring in any one mill is reasonably constant. The dilution occurring may be represented by "P," that is, P equals the concentration of caustic alkalinity in the black liquor leaving the second stage divided by the concentration of caustic alkalinity in the liquor after dilution. If the volume of black liquor charged to first stage treatments is "Q" gallons per 100 lbs. of O. D. wood, and the maximum amount of caustic alkalinity to be charged in this stage is "R" % NaOH/O. D. wood (determined as described above) then the caustic alkalinity in the black liquor charged should not exceed  $R/Q$  lbs. of NaOH per gallon, i. e.  $100R/Q$  lbs. NaOH per 100 gallons. Thus, the conditions of cooking must be controlled by increasing or decreasing the soda charge in the second stage so that the concentration of caustic alkalinity in the black liquor at the completion of this stage does not exceed  $(100R/Q) P$  lbs. NaOH per 100 gallons.

The concentration of caustic alkalinity at the completion of the second stage increases linearly with increases in the soda charge used in the second stage if the pulp produced has the same permanganate number and the amount of soda absorbed in the first stage is constant. Hence with increasing soda charge in the second stage, the time of cooking required is decreased and the caustic alkalinity in the black liquor from such treatment increases. The optimum conditions for two stage cooking will thus vary with different woods, but are such that the second stage cooking time is as short as possible, the lower limit being determined by the above mentioned preferred limitation on the caustic alkalinity of the black liquor effluent from the second stage.

## 13

## Example 7

EXPLANATION OF APPLICATION OF FORMULA  
IN EXAMPLE 6

The maximum quantity of caustic soda which can be added as white liquor in the second stage of the process described in Example 6 is calculated from the above mentioned formula as follows:

For the neutralization of 80% of the alkali in the first stage treatment an alkali charge of about 10% NaOH O. D. wood (see Figure 3 Graph B can be used. The term R of the formula is therefore 10.

The volume of black liquor charged to the first stage treatment was 9000 gallons and the amount of wood charged was equivalent to 30,000 lbs. O. D. wood. The term Q (gallons black liquor per 100 lbs. O. D. wood) is therefore 30.

The dilution factor P (concentration of caustic alkalinity in the black liquor leaving the second stage divided by the concentration of caustic alkalinity in the liquor after dilution) equals  $40/23$  or 1.7.

Hence the caustic alkalinity of the black liquor discharged from the second stage treatment should contain less than  $RP/Q$  lbs. NaOH per gallon, i. e. .563 lb. NaOH per gallon, or 56.3 lbs. NaOH per 100 gallons.

Now, the quantity of liquor present in the wood at the conclusion of the first stage was 4500 gallons, and the quantity of liquor to be added to the second stage was 7000 gallons making a total of 11,500 gallons. Of this 1800 gallons was evaporated during blowing of the digester, leaving 9700 gallons. This liquor must contain less than 56.3 lbs. NaOH per 100 gallons, that is, less than 5540 lbs. NaOH.

The residual liquor in the wood after the first stage (4500 gallons) contained 3.0 g. p. l. as NaOH, i. e. a total of 135 lbs. NaOH. The black liquor make-up added for the second stage contained 23 g. p. l., and the white liquor 120 g. p. l.

If  $x$  equals the maximum volume of white liquor chargeable to the second stage, in gallons, the maximum quantity of NaOH (in lbs.) to be charged to the second stage will be

$$135 + 23 \frac{(7000-x)}{100} + \frac{120x}{100}$$

Of this 8% NaOH is to be neutralized by the wood in the second stage, i. e. 8% of 30,000 lbs. or 2400 lbs. Hence the maximum residual free NaOH (in lbs.) to be present in the liquor from the second stage is

$$135 + 23 \frac{(7000-x)}{100} + \frac{120x}{100} - 2400$$

By the formula, this maximum quantity is 5540 lbs. Hence

$$135 + 23 \frac{(7000-x)}{100} + \frac{120x}{100} - 2400 = 5540$$

i. e.  $x = 6328$  gallons.

The quantity of NaOH to be added as white liquor for the second stage treatment must therefore be less than

$$\frac{6328 \times 120}{30000} = 25.3\% \text{ NaOH/O. D. wood}$$

As the example shows, the amount of alkali added was 16% NaOH/O. D. wood and the con-

## 14

centration of free NaOH in the black liquor was 23 g. p. l., both of which results are less than the maximum allowed, so that not less than 80% of the soda charged to the first stage will be neutralized in subsequent cooks where this method of control is exercised.

I claim:

A two-stage alkaline pulping process for the treatment of non-coniferous woods for the production of paper pulp consisting essentially in introducing a charge of wood chips into a digester, adding to the digester black liquor from a previous second stage cooking treatment in such quantity as to provide between 30 and 50 gallons per 100 pounds oven-dry wood, the alkalinity of the black liquor being equivalent to between 15 and 35 grams of active caustic soda per liter, heating the charge to a temperature between 160° C. and 175° C. with the digester closed except when gassing to remove non-condensable gases, maintaining the charge in such temperature range for a period between 6 and 30 minutes sufficient to substantially neutralize the natural acidity of the wood while neutralizing 80% to 100% of the caustic alkalinity of said black liquor, discharging the substantially exhausted liquor from the digester, then without any intervening treatment of the wood adding to the digester a digestion liquor consisting of white liquor and black liquor, the quantity and alkali concentration of the white liquor being such as to provide an effective alkali charge (expressed as NaOH) of 15 to 20 pounds per 100 pounds oven-dry wood and the total quantity of the digestion liquor added being between 15 and 35 gallons per 100 pounds oven-dry wood, original charge, heating the charge to a temperature between 160° C. and 175° C. with the digester closed except when gassing to remove non-condensable gases, maintaining the charge at a temperature in said range for a period of one to five hours, discharging the pulp and liquor from the digester, and recovering the black liquor for use in a subsequent first-stage treatment.

ARTHUR RAYMOND SLOMAN.

## References Cited in the file of this patent

## UNITED STATES PATENTS

| Number       | Name            | Date          |
|--------------|-----------------|---------------|
| 50 1,690,954 | Spencer         | Nov. 6, 1928  |
| 1,882,391    | Morterud        | Oct. 11, 1932 |
| 1,949,669    | Wells           | Mar. 6, 1934  |
| 2,047,314    | Dreyfus         | July 14, 1936 |
| 55 2,101,253 | Gunther et al.  | Dec. 7, 1937  |
| 2,190,193    | Richter         | Feb. 13, 1940 |
| 2,247,204    | Schorger et al. | June 24, 1941 |
| 2,292,390    | Meiler          | Aug. 11, 1942 |
| 2,466,290    | Wells           | Apr. 5, 1949  |

## OTHER REFERENCES

Wells: Article in Paper Trade Journal, Nov. 9, 1944, pp. 30-36 (page 31 pertinent).

Wells: Article in Paper Trade Journal, Oct. 30, 1947, pp. 42-47 (page 43 pertinent).

Davis: Article in Technical Association Papers, Series XVII, Sept. 1933, pp. 330-343 (pp. 336-7 pertinent).

Wood Chemistry by Wise, published by Reinhold Publishing Corp., New York, p. 716 (1944).